

J. F. O'CONNOR,  
ANTIFRICTION ROLLER AND PROCESS OF MAKING SAME,  
APPLICATION FILED JAN. 2, 1917.

1,273,909.

Patented July 30, 1918.



WITNESSES:

Wm. Geiger  
George A. Bishop

INVENTOR.  
John F. O'Connor  
BY George A. Bishop  
his ATTORNEY.

# UNITED STATES PATENT OFFICE.

JOHN F. O'CONNOR, OF CHICAGO, ILLINOIS, ASSIGNOR TO WILLIAM H. MINER, OF CHAZY, NEW YORK.

## ANTIFRICTION-ROLLER AND PROCESS OF MAKING SAME.

1,273,909.

Specification of Letters Patent. Patented July 30, 1918.

Application filed January 2, 1917. Serial No. 140,036.

To all whom it may concern:

Be it known that I, JOHN F. O'CONNOR, a citizen of the United States, residing at Chicago, in the county of Cook and State of Illinois, have invented a certain new and useful Improvement in Antifriction-Rollers and Processes of Making Same, of which the following is a full, clear, concise, and exact description, reference being had to the accompanying drawings, forming a part of this specification.

This invention relates to improvements in anti-friction rollers and process of making same.

The object of my invention is to provide a novel form of anti-friction roller and more particularly adapted for railway car side bearings, and process of making the same and wherein is employed an inner bushing of one form of cast material and an outer section of cast material of a different kind from the bushing, the construction of the parts and the process being such that the outer material is chilled from within during the casting process and without the necessity of external chills.

In the drawing forming a part of this specification, Figure 1 is an elevational view of a well known type of roller side bearing for railway cars, showing one use for my improved anti-friction roller. Fig. 2 is a transverse sectional view of the improved roller, taken on the line 2-2 of Fig. 3. And Fig. 3 is a longitudinal section of the roller illustrated in Fig. 2. Figs. 4 and 5 are views corresponding to Figs. 2 and 3, Fig. 4 being taken on the line 4-4 of Fig. 5 and Fig. 5 on the line 5-5 of Fig. 4, but illustrating another embodiment of the invention. Figs. 6 and 7 are views corresponding respectively to Figs. 2 and 3, but illustrating a still further embodiment of the invention, Fig. 6 being taken on the line 6-6 of Fig. 7. Figs. 8 and 9 are also views corresponding respectively to Figs. 2 and 3, but illustrating a fourth embodiment of the invention, Fig. 9 being taken on the line 9-9 of Fig. 8.

Referring first to the construction illustrated in Figs. 1, 2, and 3, 10 denotes a base casting of a roller side bearing for railway cars, which is adapted to be riveted to the truck bolster 11 thereof. Mounted in the base casting 10 is a rocking cradle 12 and carried by the cradle 12 is an anti-friction roller A

which rotates about an axle 13, the axle being supported at its ends in the cradle 12.

It is desirable to manufacture the anti-friction rollers at the least possible expense and at the same time provide a hard wearing outer surface and an inner wearing surface on the axle which will be substantially self-lubricating. Another desirable feature of anti-friction rollers of the type indicated is the avoidance of case-hardening and the use of chill molds, inasmuch as the expense of manufacture is thereby materially decreased.

In carrying out my invention, I first provide a cast bushing for the roller and then cast around the bushing the outer portion of the roller, at the same time employing means disposed around the bushing for internally chilling the outer portion of the roller during the casting process thereof.

In the arrangement illustrated in Figs. 2 and 3, 20 denotes a cylindrical hollow bushing which, in actual practice, will preferably be made of malleable iron. By employing malleable iron, all the sand and scale usually found on an ordinary casting is removed by the annealing process, thus leaving a casting the surface of which is smooth and free from foreign matter. Furthermore, by employing a malleable bushing, the same is substantially self-lubricating with respect to the axle on which the roller is mounted on account of the graphitic carbon in the malleable casting. In carrying out my invention the malleable bushing 20 is preferably provided with a series of circumferentially extending integral flanges 21, the flanges 21 being extended outwardly toward the surface of the finished roller so that said flanges will act as efficient chills when the outer portion 22 of the roller is cast therearound. In actual practice, the outer section of the roller 22 will be formed of white iron which will be sufficiently hardened due to the internal chilling by the flanges 21 during the casting process. It is furthermore obvious that the flanges 21 securely interlock the bushing and the outer portion 22 of the roller. An additional advantage resulting from the use of a malleable iron bushing resides in the fact that no "slag" will be formed at the junction between the bushing and the outer metal 22 since all sand and scale will have been removed from the bushing during the annealing process.

In the construction illustrated in Figs. 4 and 5, 120 represents the inner malleable iron bushing having a series of longitudinally and radially extending ribs or flanges 5 121 which, when the outer section 122 of white iron is cast therearound, will be embedded in the white iron and thus effectively chill the latter during the casting process.

In the construction illustrated in Figs. 6 10 and 7, 220 represents the malleable iron hollow bushing which, before the outer section 222 of white iron is cast therearound, has slipped thereover a coil of steel or iron wire 221 which acts as the chilling means for the 15 outer white iron 222.

In the construction illustrated in Figs. 8 and 9, 320 represents a central hollow bushing of malleable iron, 322 the outer section of white iron cast therearound, and 321 a 20 series of rods or bars disposed circumferentially around the bushing and parallel to the axis thereof for chilling the white iron 322.

From the preceding description, it will be seen that the anti-friction roller which I 25 have produced may be cheaply manufactured by a very simple process and at the same time obtaining a bushing which is substantially self-lubricating and an outer bearing surface of hardened material without 30 the use of chill molds.

Although I have herein shown and described different embodiments of the invention, the same are merely illustrative and I contemplate all changes and modifications 35 that come within the scope of the claims appended hereto.

I claim:

1. As an article of manufacture, an anti-friction roller adapted for use in side bear-

ings and the like, said roller comprising a 40 central hollow bushing of malleable iron, an outer surrounding portion of white iron, and means disposed around the circumference of said bushing and embedded in said white iron adapted to act as chills for the 45 white iron during the casting of the latter.

2. The herein described process for making an anti-friction roller adapted for use in side bearings and the like which consists, in providing a hollow bushing of malleable iron, providing means disposed around said bushing adapted to act as chills, and casting the outer portion of the roller of white iron around said bushing and with said means 55 embedded therein.

3. As an article of manufacture, an anti-friction roller adapted for use in side bearings and the like, said roller comprising an inner bushing centrally and axially recessed, said bushing being formed of malleable iron 60 and having a plurality of circumferentially extending integral flanges, and an outer section of white iron cast around the bushing with said flanges embedded therein.

4. The herein described process of making 65 an anti-friction roller adapted for use in side bearings and the like which consists, in first providing a malleable iron bushing having an axially extending recess and a plurality of integral, circumferentially extending flanges, and then casting about said bushing a section of white iron with said 70 flanges embedded therein.

In witness that I claim the foregoing I have hereunto subscribed my name this 29th 75 day of Dec. 1916.

JOHN F. O'CONNOR.